

April 2, 1940.

**E. L. HOFFMAN**

2,195,989

## METHOD OF PREVENTING CORROSION IN PIPE LINES

Filed Sept. 3, 1937



**INVENTOR**

INVENTOR  
*Edward L. Hoffmann*  
BY  
*Alphonse J. Buchbinder*  
ATTORNEY

## UNITED STATES PATENT OFFICE

2,195,989

METHOD OF PREVENTING CORROSION IN  
PIPE LINESEdward L. Hoffman, New York, N. Y., assignor to  
Socony-Vacuum Oil Company, Incorporated,  
New York, N. Y., a corporation of New York

Application September 3, 1937, Serial No. 162,303

5 Claims. (Cl. 196—4)

5 Pipe lines used for the transportation of gasoline and similar light petroleum fractions have been found to suffer from corrosion which is particularly severe along the bottom portion of their internal surfaces, resulting in the formation of a film of iron oxide which is dislodged at frequent intervals and carried away in the flowing stream of oil. Not only does this constant formation and dislodging of rust corrode the pipe at a highly accelerated rate, but the rust so carried away must be removed, at considerable expense, from the product in which it is suspended. This corrosion of the interior of the pipe is not spread evenly over the surface thereof but appears 10 mainly as a channeling along the bottom of the pipe, requiring retirement of the pipe from service long before the remainder of the pipe walls have deteriorated to any substantial degree.

15 It is an object of this invention to provide a method for preventing this specific form of corrosion in pipe lines carrying light petroleum fractions, and to provide a means of avoiding the deterioration of product caused by the suspension therein of products of corrosion removed from the pipe walls. A further object is to provide apparatus for carrying out such a method.

20 This invention is based upon the discovery that corrosion of this type, with its formation and subsequent carryover of rust and the like, may be prevented entirely by a method involving careful control of the water content of the petroleum fractions, particularly the gasoline, to be pumped through the pipe line, in proportion to the temperatures to be encountered while the petroleum fraction remains in the pipe. In the 25 following discussion, gasoline is taken as exemplary of such petroleum fractions.

20 Gasoline, even when free of physically admixed water which may be detected visually, still has in it some dissolved water. The amount of this water varies with the temperature and to some degree with the nature of the gasoline. Due to the history of gasoline in the petroleum refinery, in which it is often in contact with water, 40 gasoline shipped therefrom is saturated with water, up to the solubility of water in gasoline existing at the lowest temperature encountered by the gasoline in storage prior to shipment. For example, a gasoline of usual type at a temperature 45 of about 70° F., will contain about 0.0080% by weight of water. The same gasoline, when cooled to about 40° F., will contain only about 0.0040% by weight of water, thus having precipitated in the neighborhood of about one-quarter of one 50 pound of water per 1000 gallons of gasoline. In

5 pipe lines, where the daily quantity of gasoline handled is in quantities of the nature of 300,000 gallons and upwards of gasoline per day, although the net temperature change from storage to line condition is slight, there is a sufficient precipitation of water due to this condition to give an appreciable though small separation of water. It has been discovered that this water does not remain dispersed in the gasoline but appears to migrate along the bottom of the pipe 10 in the form of beads, droplets, or small streams. Likewise, the gasoline, or any other petroleum product, is always more or less saturated with oxygen, up to the limit of its solubility in the oil. It has been determined that the corrosion is caused by the combined action of moisture and oxygen, localized in those areas of the internal surface of the pipe exposed to such separated water.

15 In accordance with this invention this corrosion is prevented, and the attendant formation 20 of rust and its dispersion in the oil is likewise prevented by a suitable pretreatment of the light petroleum fraction, under controlled conditions to reduce the dissolved water content of the gasoline to such values that it will not precipitate 25 in the pipe line under the temperature conditions obtaining therein.

20 It must be understood that this benefit may be obtained only by control of the water dissolved 30 in the gasoline, or other oil, as distinguished from other water which might be associated with the oil, either as a separate phase, or as an emulsion. In short, the oil must not only be "dry", that is, entirely free from admixed or emulsified water 35 of the kind which can be removed by the common processes used for such purposes, but it must additionally have a substantial amount of its dissolved water removed. Any "dehydrating" process (using that term in the manner now common in the art), which finally draws water 40 and oil separately from some point where they exist side by side as two phases, must necessarily provide oil which, while free of discrete water, is saturated with dissolved water, and obviously 45 would be entirely useless for the practise of this invention. Therefore, in this specification, and in the claims, when the term dehydration is used, it is used in the strict sense, meaning the removal of dissolved water.

50 To understand this invention, reference is made to the attached drawing, wherein pipe 1 contains oil to be treated, 2 and 3 are chambers containing a dehydrating chemical, and 4 is an outflow pipe for treated oil. Oil entering through

5

10

15

20

25

30

35

40

45

50

55

pipe 1 is diverted through pipe 5 to flow through chamber 2 and be dehydrated therein, leaving by pipe 6 to enter pipe 4 for delivery to the transportation system. When the dehydrating chemical in chamber 2 has been sufficiently saturated with water, the oil is diverted to chamber 3 by pipe 7, returning to pipe 4 through pipe 8. The dehydrating chemical may be regenerated by means of heating under vacuum, and for this purpose the chamber is provided with internal steam coils, 20 and 23, to which steam is led through pipes 16 and 18 and from which condensate is removed by pipes 17 and 19. Vapors from regeneration are disposed of through pipes 20 and 21 which lead to a barometric condenser or other convenient vacuum device not shown. Each chamber is provided with a bottom draw pipe, 14 and 15, through which settled water, if present, may be withdrawn. Also, 14 and 15 are connected by pipes 25 and 26 to the vacuum device, in order that if necessary, vacuum may be applied to either end of the chambers. Since many products presented for transportation have higher boiling points, such as kerosene, and others, such as dyed gasolines, leave dye on the dehydrating chemical which would be taken by the next batch of oil, it is preferable to wash the chemical bed with a solvent as a portion of the regeneration step. This solvent may be introduced by pipe 9 through pipes 10 or 11, and removed by pipes 12 and 13. The solvent would preferably be a white petroleum product of low boiling point, such as undyed gasoline. If the treated oil has been kerosene or heavier, this light solvent will dissolve and displace it upon the chemical and will itself be volatilized readily in regeneration, leaving the regenerated chemical oil-free as well as water-free. Steam lines 24 and 25 are used for a purpose hereinafter explained.

The dehydrating chemical may be of any type capable of selectively removing dissolved moisture from oil and capable of convenient regeneration. Those most convenient to use are the adsorbent activated solids, such as activated alumina, "silica gel," various activated solid "gels," charcoal, some clays, and the like. Of these the medium at present preferred is activated alumina.

The dehydration of the petroleum fraction is carried to that point at which no moisture will separate at the temperature to be encountered in the pipe line transportation system. That is to say, the dissolved moisture content is reduced to a value less than the saturation value for the expected pipe line temperature.

The control of degree of dehydration may be accomplished in either of two convenient methods. Freshly saturated or regenerated chemical will remove a high proportion of the water dissolved in the gasoline, say around 70%, for example. Relatively spent chemical will remove much less, say 15% to 10% for example, and the proportionate amount removed decreases progressively as the relative "age" of the chemical, between regeneration, increases. Now, the proper amount of reduction, dependent upon the degree of saturation, the storage temperature of the oil, and the temperature to be expected in the pipe line is between these figures, ranging usually around 20 to 30% reduction. The degree of dehydration of the total oil can be controlled by sending only a portion of it through a relatively fresh chemical, securing a high proportional dehydration thereon, and blending back.

For example, with a charge of chemical capable of effecting a 60% reduction in dissolved water on the gasoline under specific conditions, and a desired reduction of only 30%, half of the gasoline could be treated and when blended with the untreated half, the desired condition would be obtained. A more convenient method, however, and in fact, the one which is preferred, is to have several dehydrating chambers as shown, the oil being passed in parallel streams through several and the streams being divided among them to arrive at the desired result. For example, with three chambers, one capable of 75% reduction, one of 50% reduction, and one of 25% reduction, with 50% overall reduction desired, then equal streams could pass through each chamber and the blended product be as desired. At the same time, a separate chamber would be undergoing regeneration, and as the efficiency of the three in use decreased toward limiting operation, the one most spent could be isolated for regeneration, and the regenerated chamber placed on stream.

The amount of water picked up by the chemical is of course dependent upon the nature of the chemical. For activated alumina, the alumina will adsorb about 10% of its weight of water before requiring regeneration.

Regeneration details will depend somewhat upon the particular chemical used. In general for the solid adsorbents and "gels" it may be accomplished by heating with coils 22 and 23 together with evacuating, or by introducing steam, preferably superheated, through 24 and 25, with or without heating by 22 and 23. Superheated steam, when used, is followed by introducing heated air through the same means, to complete drying of the chemical. As pointed out previously, the final water content of the oil is dependent upon the conditions to be met in the pipe line. Under normal conditions, in the case of gasoline, the corrosion may be reduced substantially by reducing the water content of the gasoline to from about 0.0030 per cent by weight, to about 0.0060 per cent by weight, the lower concentrations being used concurrently with lower temperatures of the ground through which the pipe line is operated, and corrosion may be entirely prevented by reducing the water content of the gasoline to a value not substantially in excess of from 0.0020 to 0.0040 by weight.

A convenient method of determining whether or not the gasoline has been dehydrated to a proper degree, is to dehydrate it previous to its entry to the pipe line, to such a degree that it does not thereafter decrease in water content during its passage through the pipe line, as may be determined by examinations of samples taken at points further along in the piping system or at the point of delivery at the end of the pipe line.

While certain numerical data have been given herein they have been set forth only by way of example, and the invention is not limited thereto or thereby, but subject only to those limitations expressed in the claims.

I claim:

1. A method of controlling internal corrosion of pipes carrying light petroleum fractions which fractions are initially entirely free of water other than dissolved water comprising passing parallel streams of oil containing dissolved water through a plurality of chambers each containing a water adsorbent material of a differing degree

of activity, removing dissolved water from said oil during the passage through said chambers, blending said streams to secure a total product of a desired degree of partial dehydration, and 5 passing said total product through the pipes.

2. A method of preventing internal corrosion of pipes carrying light petroleum fractions which 10 fractions are initially entirely free of water other than dissolved water comprising reducing the dissolved water content of the oil, before introduction to the pipe; at least to such an extent that water will not be precipitated therefrom under conditions encountered during its passage through the pipe.

15 3. A method of controlling internal corrosion of pipes carrying gasoline which gasoline is initially entirely free of water other than dissolved water comprising reducing the dissolved water content of the gasoline, before entry to the pipe, to a quantity not substantially in excess of from about 0.0030 to about 0.0060 percent by weight.

4. A method of preventing internal corrosion of gasoline-carrying pipe lines by oxidation re-

actions comprising reducing the entire water content of the gasoline, including free water content and dissolved water content of the gasoline, before entry to the pipe, to a quantity not substantially in excess of from about 0.0020 to about 5 0.0040 percent by weight.

5. In the transportation of light petroleum distillates through a pipe line characterized by the fact that said pipe line tends, upon passage of normally refined distillate therethrough, to 10 deteriorate excessively with resultant contamination of the distillate; the method of inhibiting deterioration of said pipe line and contamination of said distillate which comprises effecting the removal of water from said light petroleum distillate including the removal of a substantial portion of dissolved water contained therein to an extent such that the dissolved water content is reduced to a quantity not substantially in excess of about 0.0060% by weight and thereafter introducing said distillate of reduced water content to said pipe line.

EDWARD L. HOFFMAN.